

# UNITED STATES PATENT OFFICE.

AUGUST RAHT, OF SAN FRANCISCO, CALIFORNIA.

## DESILVERIZING LEAD BULLION.

No. 826,114.

Specification of Letters Patent.

Patented July 17, 1906.

Application filed October 11, 1905. Serial No. 282,277.

*To all whom it may concern:*

Be it known that I, AUGUST RAHT, a citizen of the United States, residing at San Francisco, in the county of San Francisco and State of California, have invented certain new and useful Improvements in Processes of Desilverizing Lead Bullion, of which the following is a specification.

This invention relates to the treatment of lead bullion—that is, an argentiferous or auriferous alloy of lead; and its object is to render a more speedy and effectual separation of the lead from the precious metals.

After the bullion has been freed of its copper, antimony, and arsenic in a "softening" furnace metallic zinc is added and stirred therein, as customary, to cause the contained gold and silver, for which it has an affinity, to rise to the surface in the form of a scum containing more or less lead, according to the character of the alloy and the manner of carrying out the process. This scum or zinc skin is skimmed off from the liquid lead by means of perforated ladles and undergoes further treatment by retorting off the zinc and cupeling to eliminate the lead, and thus obtain the silver and gold.

According to my invention a small quantity of sal-ammoniac or "chlorid of ammonium," as it is usually termed, or another similar salt is added shortly after the zinc has been introduced and thoroughly stirred with the molten metals and effects the more complete separation of the lead from the scum than is possible by the mechanical means alone above referred to. This supplementary step in the smelting process not only thus reduces the bulk of scum to be operated upon, but likewise causes it to be in a "drier" state—*i. e.*, containing less lead, and consequently more easily and cheaply treated in the following refining processes.

While my invention is a supplemental step to the various aforementioned customary ones, the additional cost is so slight as to be 45 insignificant when the resulting economy in the retorting and cupeling is considered. The amount of the ammoniacal salt for a given quantity of the metal will vary according to the requirements in each particular 50 case; but ordinarily one pound of the same will suffice for ten tons of bullion.

Having thus explained my invention, what I claim as new, and desire to secure by Letters Patent, is—

1. The treating of lead bullion while in a molten state consisting in adding zinc thereto and then adding sal-ammoniac for the purpose of causing a more ready and complete separation of the lead therefrom. 55

2. The process of treating lead bullion consisting in adding zinc to a molten mass thereof, then adding sal-ammoniac, then stirring the mixture so as to separate from the scum which is formed by the addition of the zinc a 65 portion of the lead contained in the scum.

3. The herein-described improvement in the process of desilverizing lead bullion, which consists in heating an argentiferous alloy of lead to melt the same, then adding metallic zinc to cause the separation of a portion of the lead from the more precious metals, and then adding sal-ammoniac to such incompletely-separated mass to effect a further elimination of the remaining lead therefrom. 75

In testimony whereof I affix my signature in presence of two witnesses.

AUGUST RAHT.

Witnesses:

PIERRE BARNES,  
C. F. WHITTLESEY.